

# UNITED STATES PATENT OFFICE.

MARK W. MARDSEN, OF PITTSBURG, PENNSYLVANIA, ASSIGNOR OF ONE-THIRD TO ALEX. MATCHETT, OF SAME PLACE.

## PLASTERING COMPOUND.

SPECIFICATION forming part of Letters Patent No. 269,219, dated December 19, 1882.

Application filed October 13, 1882. (No specimens.)

*To all whom it may concern:*

Be it known that I, MARK W. MARDSEN, of Pittsburgh, in the county of Allegheny and State of Pennsylvania, have invented a new and useful Improvement in Plastering Compounds; and I do hereby declare the following to be a full, clear, and exact description thereof.

My invention is directed to the production of a plaster or plastering compound which will be more adhesive, more elastic, warmer, tougher, lighter, and cheaper than ordinary plaster, and which can be used over again. I obtain such a plaster by a composition of paper or wood pulp, clay or mineral powder, and paste or sizing. The paper or wood pulp is the same as that used by paper-manufacturers in the manufacture of paper or of straw-board. For ordinary plastering the vegetable pulp is of the cheapest kind. The mineral powder used is made of soapstone, terra-alba, or other suitable clay. The paste or sizing used are of the cheaper kinds used by paper-hangers, calciminers, and whitewashers. For finer work the better and more expensive varieties of these materials are used.

I can make my improved plaster either for hard or for soft, pliable, or elastic walls. For hard walls I prefer to use the following or about the following proportions, viz: vegetable pulp, one-third; mineral powder, one-half; sizing, one-sixth. These ingredients are placed together in a box and mixed with sufficient water to give them the consistency of mortar. It is then applied to the wall in the usual way.

For soft or elastic walls I use the following or about the following proportions, viz: vegetable pulp, three-fourths; mineral powder, one-eighth; sizing, one-eighth. If it is desired to render the wall fire-proof, I add a small percentage of common salt or equivalent sub-

stances—such as soda or pearlash—which, when exposed to the heat caused by a fire or against the wall, will produce an extinguishing-gas. Coloring-matter may also be added if it is desired to color or tint the wall. The 45 vegetable pulp which I prefer to use is dry wood pulp, because it mixes up better and smoother than other pulps, and is of a fine adhesive body. The mineral powder gives body to the mass and acts as a hardener.

The advantages of my improved plaster are that it is cheaper than the ordinary plaster, as it does not require to be laid on the wall so thick. It is warmer, because it is a better non-conductor. It is more healthful, because no animal hair is used in its composition. It is more tenacious, and, being of a homogeneous, fibrous, tough structure, will not chip or scale off, and by grinding it up it can be used over again.

I am aware that it has been proposed to use 60 vegetable fiber in connection with lime, putty, and other ingredients in the manufacture of non-conducting boiler-coverings, fire-brick, roofing-tile, and similar uses, and I make no claim for any such things; but

What I do claim is—

1. A plastering compound for the walls and ceilings of houses, composed of vegetable pulp, mineral powder, and sizing, substantially as and for the purposes described.

2. A plaster composed of vegetable pulp, mineral powder, sizing, and salt, substantially as and for the purposes described.

In testimony whereof I have hereunto set my hand this 5th day of October, A. D. 1882.

MARK W. MARDSEN.

Witnesses:

T. B. KERR,  
J. K. SMITH.